

## UNITED STATES PATENT OFFICE

2,171,513

PROCESS FOR TREATING FABRICS AND  
LIKE MATERIALS TO PRODUCE EFFECTS  
THEREIN AND PRODUCTS THEREFROM

Georges Heberlein, Wattwil, and Ernst Weiss,  
Wattwil, Bunt, Switzerland, assignors to He-  
berlein Patent Corporation, New York, N. Y., a  
corporation of New York

No Drawing. Application February 13, 1936, Se-  
rial No. 63,808. In Germany February 15,  
1935

6 Claims. (Cl. 8—114)

This invention relates to a process for pro-  
ducing pattern fabrics and products therefrom.

One of the objects of the invention is to pro-  
vide simple and novel processes for the produc-  
tion of pattern crepe-effects, pattern translucent  
5 or transparent effects or for the production of a  
combination of both effects.

Another object of the invention is to provide  
special starting fabrics containing different kinds  
10 of yarns which enable the production of the de-  
sired finish effects. According to the invention  
the starting fabric contains at least two different  
sets or kinds of yarns, one set being of such  
character as to be substantially insensitive to  
15 swelling agents to which the other of the two  
sets of yarns is sensitive so as to give or enhance  
the desired optical contrast between the respec-  
tive areas of the fabric consisting of the two sets  
of yarns. Another object of the invention is to  
20 provide products from such processes having  
novel and improved characteristics. Other ob-  
jects will be in part obvious and in part pointed  
out hereinafter.

The invention comprises the novel products as  
25 well as the novel processes and steps of processes  
according to which such products are manu-  
factured, the specific embodiments of which are  
described hereinafter by way of examples and in  
accordance with which we now prefer to prac-  
30 tice the invention.

## Definitions

By "opened-up" or "active" yarns or fibers as  
35 herein mentioned, we mean vegetable yarns that  
have been cleansed by boiling, scouring, bleach-  
ing or the like, to the extent that all or substan-  
tially all of the natural incrustations are re-  
moved, so as to render said yarns sensitive to  
swelling agents.

40 By the term "raw vegetable yarns" or similar  
expressions as herein used, we mean vegetable  
yarns having all or a sufficient amount of their  
natural incrustations adhering to the fibers so  
as to render said fibers relatively insensitive to  
45 swelling agents, although the yarns may have  
been given mild cleansing or other treatments  
which do not materially remove their natural in-  
crustations.

By the term "effect yarns" as hereinafter used,  
50 we mean yarns which as woven are not substan-  
tially sensitive to the swelling agents applied to  
the fabrics containing such yarns.

The following relates to the production of  
crepe-like effects and translucent pattern effects  
55 and intermediate materials used therein employ-

ing scoured yarns and yarns containing natural  
incrustations.

1. TREATED YARNS COMBINED WITH RAW-INCURSTED  
YARNS(a) *Producing crepe-like effects by shrinkage*

In order to produce crepe-like effects (Crepon)  
in loose condition, it has already been suggested  
10 to weave together mercerized and unmercerized  
cotton yarn and to treat such fabric with mer-  
cerizing liquor without tension. Thereby the un-  
mercerized yarn shrinks while the mercerized  
yarn remains unshortened so that undulated ex-  
15 tensions and depressions are formed on the fab-  
ric. This old process produces very unsatisfac-  
tory results. These unsatisfactory results occur  
because the mercerized yarns are affected also by  
a second treatment with mercerizing lye.

In accordance with one aspect of the present  
invention it has now been found that improved  
20 effects can be obtained by the use of starting  
fabrics containing "opened-up" yarns and raw  
yarns of vegetable fibers to which the natural in-  
crustations still adhere. Swelling agents having a  
shrinkage effect known to the textile finisher are  
25 then caused to act on such fabric in accordance  
with the present invention so that the yarn pre-  
viously treated contracts while the crude yarn re-  
mains substantially uncontracted. If a very pro-  
nounced crepe-like effect is to be obtained, it is  
30 preferable to use alkali lyes of mercerizing  
strength. In this way there is produced a crepe-  
like effect which may take the most varied forms  
depending on the distribution in the fabric of the  
raw "effect"-yarns, that is, the yarns which ac-  
35 cording to this part of our invention are present  
initially in the fabric as raw yarn containing the  
natural incrustations. For example, the raw yarn  
may be woven to form stripes, diamonds, etc.  
Also other fabrics can be finished in the same  
40 manner, for instance knitted goods, hosiery goods,  
printed goods, etc. which consist of previously  
treated and raw vegetable yarns containing in-  
crustations may be employed.

After shrinking the fabric can be further treat-  
ed in any desired manner, namely by bleaching,  
dyeing, finishing or the like. In dyeing, "tone  
in tone" effects can be obtained since the previ-  
ously treated "opened-up" fiber has the property  
of consuming more dye than the raw fiber. The  
50 expression "tone in tone" is intended to indicate  
the effect given by such a combination of dyed  
fibers possessing different shades of color.

If this process is combined with the usual re-  
serve printing process, peculiar and manife'd ef- 55

fects can be obtained. For example the fabric prepared in accordance with the invention from previously treated and raw incrusted cotton yarn is printed locally with a gum reserve (Gummi Reserve) and after drying, is mercerized in loose condition. The yarn protected by the reserve remains unchanged so that these parts stand out as pattern effects.

The process is preferably employed with 10 ton containing fabrics, but the other natural vegetable fiber products can be used instead of cotton. It is important, however, in selecting for the "effect" yarns, such natural vegetable fibrous material as contains the natural incrusterations. The fabric may contain one kind of fiber alone or there may be an admixture of fibers so long as some of the yarns are relatively insensitive to the swelling agent.

The following examples embody the present 20 aspect of the invention as we now prefer to carry it out, but the invention is not to be restricted thereto except as indicated in the appended claims:

*Example 1.*—Cotton muslin, the base of which 25 consists of yarn previously scoured and into which effect-yarns of raw cotton containing incrusterations are woven in stripes, is impregnated with caustic soda solution of 37° Bé. at 10° C. for 3 seconds. The material is pressed and set 30 aside at room temperature for three minutes in unstretched condition. Thereupon it is washed hot at about 85° C., acidified and bleached carefully in the usual manner. Finally it is dried in loose condition. The effect produced is shown 35 by the wave-like projections of the effect-threads which impart to the fabric a crepe-like character.

*Example 2.*—Muslin woven from scoured cotton, yarn and also containing as effect yarns individual raw cotton yarns containing incrusterations woven into warp and filler in diamond shaped patterns is printed with a gum resist, for example gum arabic, locally. After the drying of the resist the fabric is mercerized without tension in accordance with Example 1, washed, 45 whereby also the resist is removed, and finished. The resist parts are set off as patterns from the checkered pattern background.

(b) *Producing transparent and translucent effects*

50 It is known that stiffened more or less transparent effects can be produced on cellulose-containing fabrics by means of various parchmentizing swelling agents. If this process is employed on fabrics in which thick yarns have been incorporated in thin fabrics for the purpose of producing a pattern, for example yarns woven in stripes or rectangular form, or if the process is employed on fabrics embroidered in figures forming denser parts of the fabrics, the resulting 55 products obtained by this old process have an ugly appearance. The thick incorporated threads become hard and brittle and bring about an excessive stiffness of the entire surface of the fabric.

60 It has now been found in accordance with this aspect of the present invention that these difficulties may be avoided if fabrics are prepared which contain on the one hand previously treated yarns, that is "opened" yarns as described 65 above, and on the other hand yarns which are substantially insensitive to swelling agents, namely raw yarns to which natural incrusterations still adhere. It has been found that the latter 70 yarns are not influenced by agents for producing 75 the stiffened more or less transparent effects.

As swelling agents for the production of these effects, there may be employed for example sulphuric acid of over 50.5° Bé. in conjunction with mercerized yarn, that is, mercerized yarn may be woven with a raw natural incrusted yarn and this material treated to produce a transparent effect in the mercerized yarn but substantially without producing such effect in the raw incrusted yarn. Caustic soda solution at low temperatures, approximately -10° C., may also be employed for the transparentizing treatment in conjunction with sulphuric acid treatment. Alternate treatments with caustic soda followed by sulphuric acid of 50.5° Bé. or over, followed by another treatment with caustic soda of mercerizing strength in the well-known manner may also be employed for producing transparentizing effect on cotton yarn which has been "opened-up", while the naturally incrusted yarn interwoven therewith remains substantially without change. Other reagents that may be used to give similar translucent effects, as is well-known, are the following agents used alone: sulphuric acid, phosphoric acid, mixed acid (nitric and sulphuric acid), caustic soda solution which has 25 been cooled down to about -10° C., zinc chloride, calcium thiocyanate, ammoniacal copper oxide and others. These reagents are employed under conditions of time, temperature and concentration which are well-known in the art, for example as shown in U. S. Patents 1,265,082 and 1,395,472.

According to the present invention the fabrics which have been treated to produce the translucent or transparent effects can, if desired, be further treated in order to render the original raw yarns containing the natural incrusterations susceptible to further treatment. For instance they can be treated to render them more absorptive to dyestuffs. Such raw naturally incrusted yarns can be "opened" up by bleaching or other opening up process described above. After the opening up of these raw yarns so that they then exist in a fabric which has been rendered more transparent or more translucent, the fabric can be treated with a shrinking agent such as caustic soda which will cause these non-transparent yarns to shrink so that a wavy effect will appear on the surface of the fabric of the transparent or translucent fabric.

50 In addition various effects can be obtained if the swelling agent for producing transparency or translucency is only caused to act locally on the fabrics by direct or resist printing. Pattern effects produced in this manner can be further changed by treating them again subsequently with swelling agents having a shrinking action as for instance caustic soda solution by which crepe-like patterns are obtained.

60 In addition combinations of simultaneous or successive local action of transparentizing agents (or agents for producing translucency) and shrinking agents can be employed. In connection with this patterns can be printed alongside of each other or on top of each other.

65 The effects mentioned can be further enriched by dyeing and color printing in any conceivable manner. Depending on the dyestuff selected there can be obtained thereby multi-stage shadings of the different colors because of the different action of the dyestuffs on the fibers treated by the transparentizing, shrinking and other swelling agents.

70 The following are specific examples of embodiments of this aspect of the invention as we

now prefer to practice it. The invention is not restricted thereto, however, except as indicated in the appended claims:

*Example 3.*—A cotton muslin fabric, the base of which consists of scoured cotton yarns containing woven stripes of coarse raw cotton yarns, and also effect yarns containing natural incrustations is treated with sulphuric acid of 53° Bé. at 12° C. for 8 seconds. Thereupon the acid is washed out, the fabric is mercerized with caustic soda solution of 28° Bé. at 15° C. The fabric is then bleached. The resultant product is a transparent fabric in which appears stripe effects, these stripes being the raw cotton which has not been transparentized due to the protective coating of the incrustations. These stripes remain soft and their presence does not tend to render the fabric more brittle. They give an optical contrast in which because of their non-transparent character, they are set off from the transparent base.

*Example 4.*—A cotton muslin fabric, the base of which consists of scoured cotton yarns and also containing woven stripes of coarse raw cotton yarns, as effect yarns, containing natural incrustations is treated with a solution of 70 parts of zinc chloride in 30 parts of water at 100° C. during 20 seconds. The fabric is then washed with cold water and finished in a frame. A similar effect is obtained as described in Example 3.

*Example 5.*—A cotton muslin consisting of scoured yarns and raw yarns as effect yarns forming a suitable design is printed with a resist of gum arabic and dried. Then it is treated with sulfuric acid of 54° Bé. during 10 seconds at 8° C. Then it is washed thoroughly, whereby also the resist is removed, and then bleached and finished. The resist parts stand out as patterns from the transparent background which is traced through by opaque designs due to the raw yarns.

*Example 6.*—A starting fabric of cotton muslin as described in Example 3 is transparentized in the same way as is pointed out in said example. The fabric is then kier-boiled and bleached and dried in a frame. Afterwards it is treated with caustic soda solution according to Example 1. The raw threads opened up by kier-boiling now shrink whereupon the transparent parts which remain substantially unchanged by the alkali treatment, assume a wavelike appearance.

## 2. UNCOATED YARNS COMBINED WITH COATED YARNS

### (a) Producing crepe-like effects by shrinkage

In accordance with this aspect of the present invention it has been found that instead of the vegetable yarns containing natural incrustations, there may be substituted yarns which have already been subjected to prior treatment, for instance bleached, mercerized or dyed yarns, but which prior to manufacture into fabric have been made insensitive or inert to the action of the swelling agents. There are suitable for this purpose natural vegetable yarns and artificial yarns of various kinds as well as yarns of animal origin.

The yarns or rayon threads which have been subjected to any desired prior treatment may be made insensitive to the action of the swelling agents in the following manner:

1. Sizing with sizing agents for instance starch, gum, tragacanth gum and the like.

2. Impregnating with water repellent agents, for instance a 6% emulsion of commercial paraffin or with an emulsion of higher fatty acid anhydrides and the like.

3. Impregnating with solutions of waxes and higher melting fats and hydrocarbons, for instance 10% beeswax in benzine; 10% Japan wax in benzine; 8% synthetic wax in benzine; rubber in benzol toluol, chlorinated rubber in toluol, 5 paraffin in benzine and the like.

4. Production of film-like or varnish-like coatings on the yarns by means of varnishes and resin-like substances, for instance cellulose esters, for example 15% nitrocellulose in alcohol+ethyl 10 acetate, solution of dimethyl urea, acetyl cellulose in acetone, and the like.

The vegetable or animal yarns or rayon yarns which have been made insensitive to swelling agents by any of the above-described methods 15 are now woven with previously treated "opened-up" yarns, that is, with yarns which are affected by swelling agents. Especially favorable results may be obtained with lustrous and dyed yarns which have been made insensitive in the manner 20 indicated above. The completed fabrics are shrunk by means of swelling agents known to the textile finisher including those mentioned above for crepe-like effects under (a). After the washing out of the swelling agent the insensitizing 25 material, depending on its nature, may either be removed or may remain in the fabric. In the latter case, if their presence for some particular purpose should prove objectionable they may be removed by a special process. In most cases, 30 however, such subsequent treatment is not necessary. The completed fabrics can be improved further by subsequent dyeing if desired. Such dyeing may be performed if desired before the insensitizing materials have been removed. 35

This process may be combined with the customary resist printing processes, briefly referred to above, to obtain manifold effects.

The following are examples of embodiments of the invention just described. The invention is 40 not limited thereto except as indicated in the appended claims:

*Example 7.*—A calico fabric, the base of which consists of scoured yarns and also containing as effect yarns woven stripes of mercerized cotton 45 yarns which have been impregnated with a solution made up from 15 parts of nitrocellulose, 57 parts of ethyl acetate and 28 parts of spirit is treated with caustic soda solution according to Example 1. Similar effects of those of Example 1 50 are obtained but the lustre of the mercerised effect threads imparts a good appearance to the finished fabric.

*Example 8.*—A cotton muslin which contains scoured cotton yarns and as effect yarns, cotton 55 yarns which have been mercerized, dyed and impregnated with a solution of 10% beeswax in benzine, is treated according to Example 1. A special effect is obtained by means of the dyed effect yarns. 60

### (b) Producing transparent and translucent effects

Fabrics containing sensitive uncoated and insensitive coated yarns prepared as in 2 (a) above 65 may also be treated with agents to produce areas of transparency or translucency along with some stiffening of the fabric. The swelling agents employed for producing these effects may be the same as those given under the title 1 (b) above. 70 The effects produced by the use of these insensitive yarns are similar to the effects described under 1 (b) above. The following are specific examples of this part of the invention, it being understood that the invention is not restricted 75

thereto, except as indicated in the appended claims:

Example 9.—A cotton muslin the base of which consists of scoured yarns and also containing effect yarns made insensitive to the action of parchmentizing agents by impregnation with an emulsion of paraffin (for example "Migasol" marketed by "Gesellschaft für chemische Industrie, Basel") is treated with sulfuric acid in the same way as described in Example 3. The effect yarns remain soft and give an optical contrast because of their non-transparent character.

3. RAW YARNS OR SENSITIVE YARNS COMBINED WITH FORMALDEHYDE CELLULOSE YARNS

15 Cellulose-containing yarns which have been suitably treated with formaldehyde show excellent resistance to swelling agents hereinbefore described and therefore may be used as the insensitive yarns. For example regenerated cellulose treated according to the copending application of Frauenfelder, Serial No. 62,994, filed February 8, 1936, is used. Two examples taken from this application are as follows:

25 A full cotton voile is treated in a jigger for 15 minutes at 50° C. in a 30% formaldehyde bath to which has been added 0.75% aluminum thiocyanate. After squeezing out the excess liquor the fabric is dried at above 120° C. for 20 minutes, 30 The fabric may be exposed to an air current or left lying around for a period until any odor of formaldehyde disappears. The fabric thus treated upon compression to test crease-resistance is smoothed out again and shows an agreeable soft feel.

A viscose spun-rayon fabric is treated in a jigger for 15 minutes at 20° C. in a bath containing 20 liter of technical solution of formaldehyde (38%) 400 grams of ammonium chloride and 80 liters of water. Excess liquor is squeezed out, the fabric is dried at 70° C. for about 15 minutes then exposed to a temperature of 120° C. during 20 minutes. Then follows a short treatment with a hot soap bath, containing about 3 grams of soap per liter. After washing out and drying the fabric is remarkably resistant to creasing. Similar yarns may replace the fabrics in the two examples mentioned, taken from said Frauenfelder application, Serial No. 62,994, to produce the desired inactive formaldehyde cellulose yarns herein referred to.

Such insensitive yarns accordingly may be employed with sensitive yarns for the production of crepe-like effects, as well as for the production 55 of fabrics having transparent or translucent areas. The formaldehyde cellulose yarns also possess a certain repelling property towards dye-stuffs.

It has further been found that cellulosic yarns 60 treated with formaldehyde as above show an excellent resistance to scouring (boiling with dilute alkalies) and even kier-boiling (boiling with dilute alkalies under pressure). They do not lose their valuable properties of not being affected by 65 the shrinking agents nor by the transparentizing agents referred to in Parts 1 and 2 of the present application. Thus when using these formaldehyde treated yarns there is no need of weaving scoured yarns or yarns otherwise opened up 70 (called "active cellulosic fibres" in this application) together with the "inactive" formaldehyde yarns, although such scoured yarns may be used if desired. These formaldehyde cellulose yarns 75 may be woven into a fabric with the raw vegetable yarns, for instance into a cotton voile or

muslin. This fabric may then be subjected to the customary bleaching process and also to alkali boilings without changing the valuable resist properties of the formaldehyde cellulose yarns. By such treatment the raw fibres are 5 opened up and are now "active" the formaldehyde fibres remaining "inactive".

A fabric thus prepared is ready for being subjected to a treatment with shrinking agents or transparentizing agents to produce similar effects 10 as described in Parts 1 and 2 of this application.

(a) *Producing crepe-like effects by shrinkage*

The following examples represent embodiments of the process just described. The invention is 15 not limited thereto except as indicated in the appended claims:

Example 11.—A raw cotton muslin, the base of which consists of raw cotton yarns and also containing effect twists of cotton treated according 20 to the example for cotton of said copending application is scoured, bleached and treated with caustic soda lye, according to Example 1. Similar effects are obtained as in Example 1. It is to be understood that no subsequent bleaching 25 occurs in this case, as it was necessary in Example 1 because of the raw effect threads.

Example 12.—A muslin web the base of which consists of raw cotton yarns and also containing viscose yarns treated according to the example for 30 viscose of said copending application is scoured, bleached and afterwards treated as described in Example 11. The effect yarns in this and in the previous example withstand scouring and bleaching without losing their reserving properties. Whereas the raw yarns, opened up by scouring shrink through the action of caustic alkali lye the effect yarns remain substantially unchanged and form wavelike projections all over the web.

Example 13.—A muslin such as used in either 40 of the Examples 11 and 12 is scoured, bleached, dried and printed with a gum resist, for example gum arabic, locally. Then it is treated according to Example 1 with mercerizing lye without tension, washed, acidified and washed again. If this fabric, which has already assumed a crepe-like character, the resist parts standing out as patterns, is now dyed three shades are obtained. The shrunk parts are dyed strongly, the resist parts somewhat less, the effect threads behaving 45 differently to different (colors) dyes.

The crepe-effects obtained are in general character similar to those secured in connection with the other processes described above.

(b) *Producing transparent or translucent effects* 55

Similarly the formaldehyde cellulose yarns may be combined as inactive cellulose yarns with active cotton or other vegetable fibrous material and thereafter treated with swelling agents, as 60 mentioned under 1 (b) above, for producing areas of transparency or translucency. The following examples represent embodiments of the process just described. The invention is not limited thereto except as indicated in the appended 65 claims.

Example 14.—A raw cotton muslin containing effect yarns of cotton treated with formaldehyde according to the example for treatment of cotton taken from said Frauenfelder application given above above-mentioned copending application is 70 kier-boiled bleached and dried in a frame. Afterwards it is exposed to sulfuric acid of 54° Bé. during 8 seconds at 10° C., washed, mercerized with tension, washed with hot water, acidified,

washed and finished in a frame. Thus the fabric is transparentized except for the effect threads which remain soft and opaque and give an optical contrast.

*Example 15.*—A raw cotton muslin containing effect threads of viscose artificial silk treated according to example for treatment of viscose taken from said Frauenfelder application given above the copending application mentioned above is 0 scoured, bleached, dried in a frame and printed with a resist of gum arabic. Afterwards it is exposed to sulfuric acid of 54° Bé. during 8 seconds at 12° C., thoroughly washed and finished. A peculiar effect is obtained due to the lustrous 5 viscose threads standing out from the unchanged resist parts as well as from the transparent background.

The products obtained in accordance with the examples just given are in general character 0 similar to those obtained in the examples above where agents for producing transparent or translucent effects are employed.

Depending on the distribution of formaldehyde cellulose threads in the fabric, various patterns 5 can be obtained. If desired direct or resist printing may be employed in conjunction with either the crepe-like effects or transparent or translucent effects. In addition combinations of both shrinking and transparentizing or rendering 0 more translucent can be employed on the same fabric. By these various steps effects can be produced which heretofore have only been possible by special expensive weaving technique or have been practically impossible to achieve.

The process employing the formaldehyde cellulose yarns is very simple and reliable. Due to the change in the dye-absorbing properties of the formaldehyde cellulose yarns, on dyeing a wide 0 range of color contrast in the fabric is obtained, some of which are different from those obtained by other processes herein described.

The formaldehyde-treated yarns may consist 5 of natural vegetable fibers as for instance cotton, linen, hemp, ramie and the like and also of cellulose-containing artificial fibers such as viscose, rayon, cuprammonium artificial silk, saponified nitro-rayon and artificial staple fibers. As basic substances for the vegetable yarns there may be employed all natural spinning fibers. The 0 fabrics prepared from the yarns may be of any kind, as for instance woven, braided or knitted fabrics and may contain both kinds of yarn, formaldehyde treated and untreated yarn, in varying proportions. That is, either the natural 5 active fiber may predominate or the formaldehyde cellulose fiber may predominate to give different effects.

In the claims where the expression "active fibers" is employed, it is intended to mean natural 0 fibers containing cellulose, e. g. cotton, linen, ramie and hemp or other natural cellulose-containing material which is capable of being shrunk or rendered more transparent or translucent, by any of the agents for such purpose 5 herein described.

The expression "inactive formaldehyde cellulose fibers" refers to fibers containing cellulose treated with formaldehyde as herein described. The expression "parchmentizing agent" as employed in the claims refers to sulfuric acid, zinc 0 chloride, or similar agent which acts on active fibers to produce a parchmentizing effect. This effect ordinarily shows translucence or transparency, usually with some stiffening of the fabric. The expression "parchmentized" is in-

tended to refer to the result of the action of such parchmentizing agent.

Subject matter not herein claimed is claimed in our co-pending application, Serial No. 252,938, filed January 26, 1939.

While the invention has been described in detail according to the preferred manner of carrying out the process, it will be obvious to those skilled in the art after understanding the invention, that changes and modifications may be 10 made therein without departing from the spirit or scope of the invention, and it is intended in the appended claims to cover all such changes and modifications.

What is claimed as new and desired to be secured by Letters Patent is:

1. A process for producing pattern fabrics which comprises treating with a swelling agent a fabric containing inactive formaldehyde cellulose fibres and active fibres woven in a pattern, the active fibres being natural vegetable fibres which are active to swelling agents, and altering the active fibres under the swelling action to form a visible pattern while the inactive fibres are substantially unaltered by said swelling action.

2. A process for producing pattern fabrics which comprises treating with sulfuric acid of parchmentizing strength, a fabric containing inactive formaldehyde cellulose fibres and active fibres woven in a pattern, the active fibres being natural vegetable fibres which have been treated to remove surface incrustations and render the fibres substantially active to the parchmentizing agent, to parchmentize the active fibres while the inactive fibres remain substantially unaffected by said agent.

3. A process for producing pattern fabrics which comprises treating with caustic soda of shrinking strength, a fabric containing inactive formaldehyde cellulose fibres and active fibres woven in a pattern, the active fibres being natural vegetable fibres which have been treated to remove surface incrustations, and render the fibres substantially active to the shrinking agent, and shrinking the active fibres under the action of the shrinking agent to produce a creping effect, while the inactive fibres are substantially unaltered by said shrinking agent.

4. A woven fabric containing cellulose yarn and formaldehyde cellulose yarn, the cellulose yarn being crepe-shrunk and the formaldehyde cellulose yarn being substantially unaffected by the shrinking agent, whereby a pattern appears in the fabric.

5. A woven fabric containing cellulose yarn and formaldehyde cellulose yarn, the cellulose yarn being parchmentized and the formaldehyde cellulose yarn being substantially unaffected by the parchmentizing agent, whereby a pattern appears in the fabric.

6. A process for producing pattern fabrics which comprises treating a fabric containing inactive formaldehyde cellulose fibres and active fibres successively with a swelling parchmentizing agent and with a swelling shrinking agent, the active fibres being natural vegetable fibres active to swelling agents and altering said active fibres by said agents to produce in some fibres shrinking and in others parchmentizing while the inactive fibres are substantially unaltered by said swelling agents.

GEORGES HEBERLEIN.  
ERNST WEISS.